

# United States Patent [19]

Baldassarri et al.

[11] 3,819,380

[45] June 25, 1974

[54] **AZODICARBONAMIDINE SALTS AS SILVER HALIDE FOG INHIBITORS**

[75] Inventors: **Agostino Baldassarri, Savona; Walter Ferro, Quiliano, both of Italy**

[73] Assignee: **Minnesota Mining and Manufacturing Company, St. Paul, Minn.**

[22] Filed: **Apr. 18, 1972**

[21] Appl. No.: **245,681**

[30] **Foreign Application Priority Data**

Apr. 29, 1971 Italy ..... 50035/71

[52] **U.S. Cl.** ..... 96/76 R, 96/109

[51] **Int. Cl.** ..... G03c 1/34

[58] **Field of Search** ..... 96/109, 76 R

[56]

## References Cited

### UNITED STATES PATENTS

|           |        |                   |        |
|-----------|--------|-------------------|--------|
| 3,023,103 | 2/1962 | Dersch et al..... | 96/109 |
| 3,655,391 | 4/1972 | Merli et al. .... | 96/109 |

*Primary Examiner*—Ronald H. Smith

*Assistant Examiner*—Won H. Louie, Jr.

*Attorney, Agent, or Firm*—Alexander, Sell, Steldt & Delahunt

[57]

## ABSTRACT

Azodicarbonamidine salts as a class inhibit fog formation in silver halide emulsions when contacted therewith.

**9 Claims, No Drawings**

## AZODICARBONAMIDINE SALTS AS SILVER HALIDE FOG INHIBITORS

This invention relates to azodicarbonamidine salts and particularly to the use of such compounds as fog and spot-inhibiting agents in silver halide photographic emulsions.

Metallic silver appearing in non-exposed areas of a silver halide photographic emulsion layer after development is commonly called "fog." This fog may be caused by the action of certain compounds in the emulsion, by the composition and the nature of the developer, by atmospheric oxidation, storage, etc. The type of packaging used for the photographic film can affect fog formation, as can the type of base upon which the silver halide photographic emulsion is spread. It is probable, for example, that a supporting polyester film contributes more greatly to fog in a silver halide emulsion layer than does a supporting cellulose ester film. The storage of emulsions at high temperatures and humidities favors fog formation.

In spite of the fact that fog may generally appear as a uniform blackening of emulsion layers, these layers often show small areas where the fog is darker or lighter than in the surrounding areas. Those small areas are commonly called "sensitization" or "desensitization" spots, or more simply "black spots" or "white spots." Such spots are often related to the presence in the emulsion layer (or in an adjacent layer) of metallic particles, such as particles of iron, copper, tin or their derivatives. These particles are, in turn, related to the type of base used (for instance polyester) or are caused by the environment wherein the material has been prepared or used.

The formation of fog and spots in silver halide photographic emulsions continues as a problem in the photographic field, and reduction of elimination of this problem is greatly to be desired.

It has now been found that fog and spots (hereinafter collectively called "fog") in silver halide photographic emulsions, can be strongly inhibited by using, as fog inhibitors, an azodicarbonamidine salt. Such compounds preferably have the formula



wherein  $R_1$ ,  $R_2$ ,  $R_3$  and  $R_4$  independently are hydrogen, alkyl or aryl, and  $X$  represents an equivalent of anion, such as chloride, nitrate, sulfate or picrate. Formula I can also be written



wherein  $R_1$ ,  $R_2$ ,  $R_3$ ,  $R_4$  and  $X$  are as given above.

In one embodiment, accordingly, the invention relates to a silver halide photographic emulsion having contacted therewith (i.e., in reactive association therewith) an azodicarbonamidine salt to inhibit fog. For example, an azodicarbonamidine salt may be mixed into

the emulsion, may be placed in a layer adjacent an emulsion layer, or may be introduced into developer baths or pre-developer baths. Preferred azodicarbonamidine salts for this purpose are those defined in Formulae I and IA above. In another embodiment, the invention relates to a method for inhibiting fog in a silver halide photographic emulsion which comprises contacting the emulsion with an azodicarbonamidine salt, preferably of the type defined in Formulae I and IA. The ability to inhibit fog in silver halide emulsions is shared by azodicarbonamidines as a class.

In another embodiment, the invention relates to novel azodicarbonamidine salts which are useful as fog inhibitors for silver halide emulsions and which are characterized by the formula



wherein  $R_1$ ,  $R_2$ ,  $R_3$  and  $R_4$  independently are hydrogen, alkyl or aryl with the proviso that at least one (and preferably two or more) of  $R_1$ ,  $R_2$ ,  $R_3$  and  $R_4$  is different from hydrogen, and  $X$  is an equivalent of anion. Formula II can also be written



wherein  $R_1$ ,  $R_2$ ,  $R_3$ ,  $R_4$  and  $X$  are as defined next above.

As will be evident from the examples below, azodicarbonamidine salts may be prepared by oxidizing, e.g., with potassium permanganate in aqueous nitric acid, an N-substituted amino guanidine obtained in a known way, e.g., by reacting an N-substituted-S-methyl isothiourea with hydrazine, or the reduction product of an N-substituted nitroguanidine with high pressure hydrogen in the presence of a platinum oxide catalyst. In another preparation method, an N-substituted-S-methyl isothiourea may be reacted in a suitable solvent, such as pyridine, with an N-substituted amino guanidine; the resulting hydrazodicarbonamidine then being oxidized to the corresponding azodicarbonamidine.

As mentioned above, azodicarbonamidine salts as a class have been found to inhibit fog in silver halide photographic emulsions. The choice of groups  $R_1$ ,  $R_2$ ,  $R_3$  and  $R_4$  will vary to some extent the fog inhibiting capacity and solubilities of compounds of the invention, and it is preferred that the alkyl or aryl groups — which may be represented by each of  $R_1$ ,  $R_2$ ,  $R_3$  and  $R_4$  in formulas I, IA, II and II A above — be limited respectively to no more than 4 and 14 carbon atoms. Although the selection of the anion  $X$  may also effect to a small extent these properties, the selection of  $X$  is not critical to the invention. Chloride (e.g., halide), nitrate, sulfate and picrate (particularly the latter) are preferred anions. The compounds of the present invention are solvent-soluble; e.g., they are soluble in the primarily polar solvents employed in photography, including, for example, water, alcohol, and dimethylformamide. The

invention may be illustrated by reference to the following non-limiting examples:

#### EXAMPLE 1

##### N,N'-dimethyl-azodicarbonamidine nitrate

Into an open 750 cc flask supplied with mechanical stirrer and a thermometer and placed on a refrigerating bath, were introduced 10 cc of water and 40 cc of 70 % nitric acid in which the reduction product of 0.1 moles of N-methyl-nitroguanidine was previously dissolved. (The reduction was performed by known procedures employing high pressure hydrogen in the presence of platinum oxide). The resulting solution was cooled to -5°C and at this temperature was slowly and carefully treated with small portions of powdered potassium permanganate. An exothermic reaction occurred with gas evolution (foaming) and the solution rapidly acquired an increasingly intense color. The permanganate addition was continued until it began to impart a dark coloration which lasted for some seconds; concurrently a yellow crystalline solid formed. The mixture was rapidly filtered and when the product was almost dry, it was washed with 100 cc of ethanol. It was dried under vacuum at 30°C. 2.05 g of very small yellow crystals were obtained, with a decomposition point of 162°C, formed by N,N'-dimethyl-azodicarbonamidine nitrate. The product, in the form of a yellow powder, was highly soluble in water, soluble in dimethylformamide, insoluble in alcohol, in acetone and in non-polar solvents.

##### Elemental Analysis:

|    | Calculated | Found |
|----|------------|-------|
| N% | 41.76      | 41.38 |
| C% | 16.95      | 17.14 |
| H% | 4.48       | 4.45  |

#### EXAMPLE 2

##### N,N'-dimethyl-azodicarbonamidine picrate

A concentrated solution of N,N'-dimethyl-azodicarbonamidine nitrate in water was treated with a slight excess of a saturated solution of picric acid to cause nearly quantitative separation of N,N'-dimethyl-azodicarbonamidine picrate in the form of very fine, short needles with an intense red color. The decomposition point was 189°C. The product was highly soluble in dimethylformamide, and slightly soluble in ethanol.

##### Elemental Analysis:

|    | Calculated | Found |
|----|------------|-------|
| N% | 28.02      | 28.22 |
| C% | 32.05      | 31.21 |
| H% | 2.67       | 2.70  |

#### EXAMPLE 3

##### N,N'-diethyl-azodicarbonamidine nitrate

Into a 750 cc covered flask, equipped with mechanical stirrer and a thermometer and placed on a refrigerating bath, were introduced 35 cc of 70% nitric acid and 35 cc of water containing in solution, the product of the reduction (obtained with high pressure hydrogen

in presence of platinum oxide) of 0.1 moles of N-ethyl-nitroguanidine. The solution was cooled to -5°C and at this temperature small quantities of potassium permanganate in powder form were added very carefully. The resulting exothermic reaction caused the formation of a large amount of foam, and the solution rapidly attained an intense yellow coloration. When almost two-thirds of the oxidant was added, a light luminous yellow solid began to separate out. At the end of the reaction the mixture was rapidly filtered nearly dry; then it was washed with 100 cc of ethanol and dried under vacuum at 35°C.

3.1 g of mother-of-pearl-like scales of a light-yellow color, formed by N,N'-diethyl-azodicarbonamidine nitrate, with a decomposition point of 113°C were obtained. The solubility was excellent in water, good in dimethylformamide, and slight in alcohol.

##### Elemental Analysis:

|    | Calculated | Found |
|----|------------|-------|
| N% | 37.83      | 37.58 |
| C% | 24.33      | 24.23 |
| H% | 5.44       | 5.41  |

#### EXAMPLE 4

##### N,N'-diethyl-azodicarbonamidine picrate

From a concentrated solution of N,N'-diethyl-azodicarbonamidine nitrate in water, by treatment with an excess of a saturated solution of picric acid, N,N'-diethyl-azodicarbonamidine picrate separated almost quantitatively as very fine, intensely red needles. The decomposition point was 154°C. The solubility of the product was very high in dimethylformamide, and slight in alcohol and in cold water.

##### Elemental Analysis:

|    | Calculated | Found |
|----|------------|-------|
| N% | 26.76      | 26.80 |
| C% | 34.33      | 34.17 |
| H% | 3.18       | 3.24  |

#### EXAMPLE 5

##### N,N'-dipropyl-azodicarbonamidine nitrate

Into a 750 cc flask equipped with mechanical stirrer and a thermometer and placed on a refrigerating bath were introduced 35 cc of 70% nitric acid and 25 cc of water containing in solution the reduction product (obtained with high pressure hydrogen in presence of platinum oxide) of 0.1 moles of propyl-nitroguanidine. The solution was cooled to -5°C and at this temperature small amounts of powdered potassium permanganate were very carefully added. An exothermic reaction occurred which produced a large amount of foam, and the solution turned rapidly became intensely yellow. During a two hour period, from about 6.5 to about 7.5 g of powdered potassium permanganate were thus added. Near the end of the reaction, a yellow, crystalline, light and fluffy solid began to separate out. Upon completion of the reaction, the mixture was rapidly filtered to a semi-dry condition and was then washed with ethanol (100 cc) and dried under vacuum at 35°C.

2.15 g of light yellow, mother-of-pearl-like small scales of N,N'-dipropyl-azodicarbonamidine nitrate were obtained.

Crystallization of the product from small volumes of hot water (90°C, 4 cc per gram of product) was rapidly performed to prevent decomposition. Mother-of-pearl-like small scales, with a decomposition point of 161°C were obtained. The solubility of the product was excellent in water, good in dimethylformamide, and slight in alcohol.

| Elemental Analysis: | Calculated | Found |
|---------------------|------------|-------|
| N%                  | 34.55      | 34.66 |
| C%                  | 29.65      | 29.93 |
| H%                  | 6.17       | 6.26  |

### EXAMPLE 6

#### N,N'-dipropyl-azodicarbonamidine picrate

To a concentrated solution of N,N'-dipropyl-azodicarbonamidine nitrate in cold water was added an excess of a saturated solution of picric acid. N,N'-dipropyl-azodicarbonamidine picrate separated almost quantitatively as very fine small needles of an intense red color. The decomposition point was 176°C. The solubility of the product was very high in dimethylformamide and slight in alcohol and in water.

| Elemental Analysis: | Calculated | Found |
|---------------------|------------|-------|
| N%                  | 25.65      | 25.60 |
| C%                  | 36.65      | 36.81 |
| H%                  | 3.66       | 3.74  |

### EXAMPLE 7

#### N,N'-tetramethyl-azodicarbonamidine picrate

Into a 750 cc flask equipped with mechanical stirrer and a thermometer and placed on a refrigerating bath were introduced 20 cc of 70% nitric acid and 20 cc of water containing in solution the reduction product (obtained with high pressure hydrogen in presence of platinum oxide) of 0.03 moles of N,N'-dimethyl-N'-nitroguanidine. The solution was cooled to -3°C and at this temperature a small amount of powdered potassium permanganate was carefully added. An exothermic reaction occurred with development of gas. A yellow solution was obtained, which was filtered (maintaining a temperature below 0°C) and treated with an excess of a saturated solution of picric acid (0.05 moles). A yellow crystalline solid separated out and was collected by filtration, dried under vacuum at 35°C and then thoroughly washed with 250 cc of diethylether.

4.5 g of very small, light-yellow needles of N,N'-tetramethyl-azodicarbonamidine picrate were obtained. The decomposition point was 203°-205°C. The solubility of the product in dimethylformamide was excellent.

| Elemental Analysis: | Calculated | Found |
|---------------------|------------|-------|
| N%                  | 26.74      | 26.49 |
| C%                  | 34.30      | 34.27 |
| H%                  | 3.17       | 3.25  |

### EXAMPLE 8

#### N,N'-diphenyl-azodicarbonamidine picrate

Into a 750 cc flask equipped with mechanical stirrer and a thermometer and placed on a refrigerating bath were introduced 21.3 g (0.01 moles) of N-phenyl-amino-guanidine nitrate, and 100 cc of 70% nitric acid and 100 cc of water to form a solution. The solution was cooled to -2°C and at this temperature, small amounts of potassium permanganate in powder were added very carefully. An exothermic reaction occurred with gas development. In two hours, 9.7 g of permanganate (0.061 moles) were added. The mixture was rapidly filtered, maintaining cold conditions, and the filtrate was treated with an excess of a saturated solution of picric acid. A red fluffy solid separated out and was collected on a vacuum filter, dried under vacuum at 30°C, and ground twice with 250 cc of ether. The mixture was filtered again. After drying under vacuum at 30°C there remained 12.3 g (equal to 34% of the theoretical yield) of a red powder, melting at 90°-95°C, with decomposition. The solubility of the product was excellent in dimethylformamide, good in alcohol and in acetone, and slight in cold water. The product was then very rapidly crystallized from boiling water. By crystallization an extremely electrifyable powder (e.g., capable of maintaining an electric charge) of a dark yellow color with a melting point of 154°C (with decomposition) was obtained. The solubility was similar to that of the raw product.

| Elemental Analysis: | Calculated | Found |
|---------------------|------------|-------|
| N%                  | 23.20      | 23.05 |
| C%                  | 43.15      | 43.09 |
| H%                  | 2.77       | 2.88  |

### EXAMPLE 9

#### N,N'-di-m-tolyl-azodicarbonamidine picrate

Into a 750 cc flask equipped with mechanical stirrer and a thermometer and placed on a refrigerating bath were introduced 30 cc of 70% nitric acid and 35 cc of water, containing, in solution, the reduction product (obtained with high pressure hydrogen and platinum oxide) of 0.05 moles of N-m-tolyl,N'-nitroguanidine. The solution was cooled to -3°C and at this temperature, small amounts of powdered potassium permanganate were added very carefully. An exothermic reaction occurred with gas development, and the solution rapidly became red. After the addition of a rather large quantity of potassium permanganate, a soft, pitchy material of an intense red color began to separate out. After addition of 4.85 g of potassium permanganate, the separated pitchy material, presumably N,N'-di-m-tolyl-azodicarbonamidine nitrate, was collected, washed with small amount of water, dissolved in 30 cc

of cold ethanol and treated with an excess of a saturated solution of picric acid. A fluffy red-orange solid was obtained which was separated by filtration, washed with cold water, dried under vacuum at 30°C, and ground twice with 200 cc of ethyl ether in a mortar. After drying, there remained 5.3 g of a yellow red powder of N,N'-di-m-tolyl-azodicarbonamidine picrate. M.P. 109°C. The solubility of the product was excellent in dimethylformamide, good in alcohol and in acetone, and slight in water.

| Elemental Analysis: |       | Calculated | Found |
|---------------------|-------|------------|-------|
| N%                  | 22.32 | 22.49      |       |
| C%                  | 44.65 | 44.90      |       |
| H%                  | 3.19  | 3.31       |       |

#### EXAMPLE 10

##### N,N'-di- $\alpha$ -naphthyl-azodicarbonamidine nitrate

Into a 750 cc flask equipped with mechanical stirrer and a thermometer and placed on a refrigerating bath were introduced 40 cc of 70% nitric acid containing dissolved 13.15 g (0.05 moles) of N'- $\alpha$ -naphthyl,N'-aminoguanidine nitrate. The solution was cooled to -2°C and at this temperature small amounts of powdered potassium permanganate were carefully added. An exothermic reaction occurred, with gas development, and the solution rapidly turned a dark red. The amount of KMnO<sub>4</sub> used was 4.85 g (0.6 moles per mole of aminoguanidine). When the reaction was almost completed, a reddish pitchy material began to separate out. After the completion of the permanganate addition, this pitchy material was separated from the mother liquor (a), washed with a small amount of water, and air-dried. It was then ground in a mortar to yield a brown-red powder of N,N'-di- $\alpha$ -naphthyl-azodicarbonamidine nitrate; M.P. 160°C, with decomposition. The solubility of the product was excellent in dimethylformamide and good in ethanol and acetone.

45

| Elemental Analysis: |       | Calculated | Found |
|---------------------|-------|------------|-------|
| N%                  | 22.34 | 22.03      |       |
| C%                  | 44.65 | 44.95      |       |
| H%                  | 3.18  | 3.33       |       |

#### EXAMPLE 11

##### N,N'-di- $\alpha$ -naphthyl-azodicarbonamidine picrate

The mother liquor (a) of Example 10 was treated with an excess of a solution of picric acid to cause separation of a red-brown precipitate of N,N'- $\alpha$ -naphthyl-azodicarbonamidine picrate. The product was collected, dried under vacuum at 30°C, washed twice with 200 cc of ether, and dried again. The product obtained decomposed at 106°C. Solubility was excellent in dimethylformamide and good in ethanol and in acetone.

| Elemental Analysis: |       | Calculated | Found |
|---------------------|-------|------------|-------|
| N%                  | 20.34 | 19.69      |       |
| C%                  | 49.45 | 49.09      |       |
| H%                  | 2.91  | 3.12       |       |

10

#### EXAMPLE 12

##### N,N'-di-(methyl,phenyl)-azodicarbonamidine picrate

N-methyl-N-phenyl-N'-aminoguanidine nitrate (11.35 g, 0.05 moles) were dissolved in 30 cc of 70% nitric acid and introduced into a 750 cc flask, equipped with mechanical stirrer and a thermometer and placed on a refrigerating bath. The temperature was brought to -3°C and kept constant while 4.85 g of powdered potassium permanganate were carefully added in small portions over about a one hour period. The addition was performed very carefully to avoid overheating from the resulting exotherm. Gas development was observed. The resulting solution was filtered cold and then treated with an excess of a saturated solution of picric acid. A reddish voluminous solid separated out and was collected by filtration, washed with a small amount of water, dried under vacuum at 30°C, then ground twice with 200 cc of ether, filtered and dried. A reddish-yellow powder of N,N'-di(phenyl,methyl)-azodicarbonamidine picrate (which may be termed N,N'-dimethyl-N,N'-diphenyl-azodicarbonamidine) was obtained. The melting point was 90°C with decomposition. The yield was 5.6 g, equivalent to 29% of theoretical. Solubility was excellent in dimethylformamide and good in alcohol and in acetone.

25

| Elemental Analysis: |       | Calculated | Found |
|---------------------|-------|------------|-------|
| N%                  | 22.34 | 22.03      |       |
| C%                  | 44.65 | 44.95      |       |
| H%                  | 3.18  | 3.33       |       |

30

#### EXAMPLE 13

##### N-ethyl-N'-phenyl-azodicarbonamidine picrate

4.92 g (0.02 moles) of N-ethyl-S-methyl-isothiourea iodide and 5.84 g (0.02 moles) of N-phenyl-N'-aminoguanidine iodide, and 20 cc of pyridine were introduced into a 250 cc flask equipped for reflux. The mixture was heated to the boil. After a few minutes it was clearly evident from the odor of methylmercaptan that the reaction had begun. Heating was continued until the development of methylmercaptan ceased. The mixture (after cooling) was poured into 200 cc of ethyl ether and the resulting pitchy material was washed several times with ether. The same pitchy material (consisting primarily of N-phenyl-N'-ethyl,hydrazodicarbonamidine iodide) was finely powdered and suspended in 50 cc of methylene chloride. A solution of 0.02 moles (3.1 g) of N-chloro-benzotriazole in 20 cc of methylene chloride were added dropwise to the suspension with stirring and cooling to 0°C. The mixture turned intensely red and an orange pitchy solid separated out. The mixture was filtered under vacuum and washed carefully with a small amount of cold ethanol

| Elemental Analysis: |       | Calculated | Found |
|---------------------|-------|------------|-------|
| N%                  | 22.72 | 22.48      |       |
| C%                  | 53.70 | 53.97      |       |
| H%                  | 4.07  | 4.25       |       |

#### EXAMPLE 11

##### N,N'-di- $\alpha$ -naphthyl-azodicarbonamidine picrate

The mother liquor (a) of Example 10 was treated with an excess of a solution of picric acid to cause separation of a red-brown precipitate of N,N'- $\alpha$ -naphthyl-azodicarbonamidine picrate. The product was collected, dried under vacuum at 30°C, washed twice with 200 cc of ether, and dried again. The product obtained decomposed at 106°C. Solubility was excellent in dimethylformamide and good in ethanol and in acetone.

45

50

55

60

65

(about 3 cc). The solid was dissolved in 15 cc of ethanol and 150 cc of a saturated aqueous solution of picric acid was rapidly added. The flaky red-orange solid which formed was collected by filtration, thoroughly washed with cold water, dried under vacuum at room temperature, washed thoroughly with ether (by grinding in a mortar) and dried again. The melting point was 148°-150°C with decomposition. Solubility was good in dimethylformamide, ethanol and acetone.

## Elemental Analysis:

|    | Calculated | Found |
|----|------------|-------|
| N% | 24.85      | 24.60 |
| C% | 39.20      | 40.51 |
| H% | 2.96       | 2.78  |

Azodicarbonamide salts are useful for prevention of fog in silver chloride, silver bromide and silver iodide emulsions and in emulsions comprising mixtures of such silver halides (such as, for example, silver bromo-iodide emulsions). The emulsions of the invention may contain various synthetical polymers as colloidal liquids in substitution for, or in addition to the commonly employed gelatin. Exemplary of such polymers are dextrane, polyvinylalcohol, polyvinylpyrrolidone, partially hydrolyzed polyvinylacetate, polyethylacrylate, polymethylmethacrylate and polyamides. The emulsions of the invention may be chemically sensitized by remelting with naturally activated gelatin, by addition of chemical sensitizers such as thiosulfate, allylthiourea, thiocyanates, thiosulphonates, etc., by employment of salts of noble metals (for example gold salts), etc. The emulsions may contain spectral sensitizers such as cyanine and mercocyanine dyes, and may contain couplers, surface active agents, hardeners, stabilizers, antifog agents, plasticizers, anti-oxidants, development accelerators and, in general, the various additives commonly used in the production of silver halide photographic emulsions. Such emulsions may be spread upon any suitable support such as polystyrene, polyester, cellulose acetate, polycarbonate, paper, glass, etc. The azodicarbonamide salts of the present invention are particularly suitable for the prevention of fog usually occurring when a polyester film support (for example, polyethyleneterephthalate) is used or when unusually rapid processes for the spreading and drying of the emulsions are used.

The incorporation of azodicarbonamide salts in silver halide emulsions may be conveniently accomplished by adding them to the emulsions during preparation thereof. Even though it is preferable that the azodicarbonamide salts be incorporated into silver halide emulsion layers, fog and spots are avoided or minimized if the salts are at least put into contact with the silver halide emulsion layers as described previously. For example, fog-inhibiting amounts of azodicarbonamide salts can be introduced into a layer adjacent to the silver halide layer in a photographic element, or can be used in solutions for photographic processing. The amounts of azodicarbonamide salts required for fog inhibition when employed in a silver halide layer or in an adjacent layer will vary depending upon the salt selected, and such elements can be determined by routine testing. When used in a photographic emulsion, it is preferred to employ from about 0.1 to

about 2.5 millimoles of an azodicarbonamide salt such as those exemplified above per gram-atom of silver.

The novel compounds of Examples 1-13 have been evaluated photographically together with previously known azodicarbonamide salts representing further examples of such salts useful as fog-inhibitors according to the present invention. These compounds are azodicarbonamide nitrate (Example 14), azodicarbonamide sulfate (Example 15), azodicarbonamide chloride (Example 16) and azodicarbonamide picrate (Example 17).

## EXAMPLE 18

15 The solubility of compounds 1-17 in common solvents used in photography (water, ethyl alcohol and dimethylformamide (DMF)) at room temperature (about 20°C) was measured. The results are schematically reported in Table 1 wherein + indicates a solubility greater than 1 per cent and - a solubility less than 0.05%.

TABLE 1

| Compound | H <sub>2</sub> O | C <sub>2</sub> H <sub>5</sub> OH | DMF |
|----------|------------------|----------------------------------|-----|
| No. 14   | +                | -                                | +   |
| No. 15   | +                | -                                | +   |
| No. 16   | +                | -                                | +   |
| No. 17   | -                | +                                | +   |
| No. 1    | +                | -                                | +   |
| No. 2    | -                | -                                | +   |
| No. 3    | +                | -                                | +   |
| No. 4    | -                | -                                | +   |
| No. 5    | +                | -                                | +   |
| No. 6    | -                | -                                | +   |
| No. 7    | -                | +                                | +   |
| No. 8    | -                | +                                | +   |
| No. 9    | -                | -                                | +   |
| No. 10   | -                | +                                | +   |
| No. 11   | -                | +                                | +   |
| No. 12   | -                | +                                | +   |
| No. 13   | -                | +                                | +   |

## EXAMPLE 19

45 A silver halide photographic emulsion of high sensitivity, containing 1.8 mole % of AgI and 98.2 mole % of AgBr, with a ratio of silver/gelatin of 1.6 was divided into several parts. One part was spread, without further treatment, on a cellulose triacetate base. To the other parts were added the compounds indicated in Table 2 in the reported quantities, and the resulting emulsions 50 were similarly spread on a cellulose triacetate base. The resulting film samples were then exposed to tungsten light and developed for 5' or 10' at 20°C in a Ferrania R-14 developer of the following composition (Ferrania R-14 developer):

|                            |         |
|----------------------------|---------|
| Metol                      | 3 g     |
| Anhydrous sodium sulfite   | 50 g    |
| Hydroquinone               | 9 g     |
| Anhydrous sodium carbonate | 50 g    |
| Potassium bromide          | 3 g     |
| Water to                   | 1000 cc |

65 Table 2 reports the results of sensitometric test performed on fresh film samples and on film samples stored respectively for 15 hours at 72°C, and at 30% R.H.

TABLE 2

| Compound No. | $\mu\text{M/M}$<br>AgX | Fresh<br>5' | Fog<br>15 h 72°C<br>5' | 30% R.H.<br>10' | Relative Sensitivity | Solvent used |
|--------------|------------------------|-------------|------------------------|-----------------|----------------------|--------------|
| —            | —                      | 23          | 30                     | 22              | 32                   | 100          |
| 14           | 100                    | 22          | 27                     | 20              | 26                   | 117          |
| 14           | 500                    | 07          | 05                     | 05              | 14                   | 71           |
| 14           | 2500                   | 06          | 06                     | 06              | 13                   | 36           |
| 15           | 100                    | 18          | 26                     | 20              | 26                   | 85           |
| 15           | 500                    | 14          | 24                     | 15              | 22                   | 85           |
| 15           | 2500                   | 06          | 12                     | 05              | 11                   | 25           |
| 16           | 100                    | 09          | 15                     | 07              | 14                   | 71           |
| 16           | 500                    | 09          | 14                     | 07              | 14                   | 71           |
| 16           | 2500                   | 05          | 13                     | 04              | 11                   | 36           |
| 17           | 100                    | 18          | 26                     | 22              | 28                   | 89           |
| 17           | 500                    | 18          | 26                     | 22              | 28                   | 89           |
| 17           | 2500                   | 14          | 22                     | 14              | 22                   | 89           |
| 1            | 100                    | 15          | 24                     | 20              | 26                   | 100          |
| 1            | 500                    | 15          | 22                     | 16              | 24                   | 96           |
| 1            | 2500                   | 14          | 20                     | 14              | 22                   | 79           |
| 2            | 100                    | 19          | 26                     | 20              | 28                   | 112          |
| 2            | 500                    | 15          | 24                     | 20              | 26                   | 100          |
| 2            | 2500                   | 09          | 13                     | 10              | 17                   | 56           |
| 3            | 100                    | 27          | 31                     | 23              | 34                   | 110          |
| 3            | 500                    | 23          | 29                     | 23              | 32                   | 110          |
| 3            | 2500                   | 18          | 28                     | 19              | 28                   | 98           |
| 4            | 100                    | 21          | 24                     | 22              | 26                   | 112          |
| 4            | 500                    | 15          | 24                     | 16              | 24                   | 96           |
| 4            | 2500                   | 12          | 15                     | 12              | 19                   | 79           |
| 5            | 100                    | 24          | 32                     | 22              | 94                   | 107          |
| 5            | 500                    | 19          | 28                     | 19              | 29                   | 91           |
| 5            | 2500                   | 18          | 28                     | 17              | 27                   | 91           |
| 6            | 100                    | 25          | 29                     | 23              | 34                   | 91           |
| 6            | 500                    | 21          | 27                     | 21              | 33                   | 59           |
| 6            | 2500                   | 19          | 27                     | 19              | 33                   | 59           |
| 7            | 100                    | 15          | 21                     | 14              | 20                   | 25           |
| 7            | 500                    | 08          | 16                     | 05              | 16                   | 10.5         |
| 7            | 2500                   | 05          | 15                     | 05              | 16                   | 16           |
| 8            | 100                    | 11          | 18                     | 08              | 19                   | 63           |
| 8            | 500                    | 09          | 18                     | 08              | 17                   | 40           |
| 8            | 2500                   | 05          | 16                     | 03              | 10                   | 11           |
| 9            | 100                    | 10          | 26                     | 08              | 18                   | 45           |
| 9            | 500                    | 07          | 18                     | 06              | 17                   | 22           |
| 9            | 2500                   | 07          | 18                     | 06              | 17                   | 10           |
| 10           | 100                    | 25          | 33                     | 25              | 35                   | 96           |
| 10           | 500                    | 23          | 29                     | 24              | 29                   | 79           |
| 10           | 2500                   | 18          | 25                     | 15              | 19                   | 79           |
| 11           | 100                    | 24          | 32                     | 27              | 34                   | 98           |
| 11           | 500                    | 22          | 29                     | 24              | 29                   | 80           |
| 11           | 2500                   | 17          | 26                     | 16              | 18                   | 79           |
| 12           | 100                    | 15          | 23                     | 09              | 25                   | 79           |
| 12           | 500                    | 08          | 19                     | 06              | 20                   | 28           |
| 12           | 2500                   | 03          | 07                     | 04              | 08                   | 5            |
| 13           | 100                    | 06          | 16                     | 26              | 35                   | 34           |
| 13           | 500                    | 04          | 10                     | 12              | 20                   | 25           |
| 13           | 2500                   | 04          | 10                     | 08              | 18                   | 14           |

## EXAMPLE 20

A high sensitivity silver halide photographic emulsion containing 1.5 mole % of AgI and 98.5 mole % of AgBr, with a ratio of silver to gelatin of 0.8 was divided into several portions. One of these portions was spread without further treatment on a cellulose triacetate base. To the other portions were added respectively the

compounds indicated in Table 3 in the reported quantities, and the resulting emulsions were spread on a cellulose triacetate base. Samples of the resulting films were then exposed to tungsten light and developed for 3' at 20°C in Ferrania R-14 developer (See Example 19). Table 3 reports the results of sensitometric tests performed on fresh film samples and on film samples respectively stored for 15 hours at 72°C and at 30% R.H.

TABLE 3

| Compound No. | $\mu\text{M/M}$<br>AgX | Fresh<br>5' | Fog<br>15 h 72°C<br>5' | 30% R.H.<br>10' | Relative Sensitivity | Solvent used |
|--------------|------------------------|-------------|------------------------|-----------------|----------------------|--------------|
| —            | —                      | 16          | 21                     | 16              | 23                   | 100          |
| 14           | 100                    | 16          | 19                     | 14              | 18                   | 120          |
| 14           | 500                    | 05          | 04                     | 04              | 10                   | 73           |
| 14           | 2500                   | 04          | 04                     | 03              | 09                   | 38           |
| 15           | 100                    | 13          | 18                     | 14              | 18                   | 88           |
| 15           | 500                    | 10          | 17                     | 10              | 15                   | 88           |
| 15           | 2500                   | 04          | 04                     | 03              | 08                   | 27           |
| 16           | 100                    | 06          | 10                     | 05              | 10                   | 70           |
| 16           | 500                    | 06          | 10                     | 05              | 10                   | 70           |
| 16           | 2500                   | 03          | 09                     | 03              | 08                   | 36           |

TABLE 3—Continued

| Compound No. | $\mu\text{M/M AgX}$ | Fresh 5' | Fog 15 h 72°C 5' | 30% R.H. 10' | Relative Sensitivity | Solvent used |
|--------------|---------------------|----------|------------------|--------------|----------------------|--------------|
| 17           | 100                 | 12       | 18               | 15           | 20                   | 90           |
| 17           | 500                 | 12       | 18               | 15           | 20                   | 90           |
| 17           | 2500                | 10       | 15               | 10           | 15                   | 90           |
| 1            | 100                 | 11       | 17               | 14           | 18                   | 100          |
| 1            | 500                 | 10       | 15               | 11           | 27                   | 95           |
| 1            | 2500                | 09       | 14               | 10           | 15                   | 80           |
| 2            | 100                 | 13       | 18               | 14           | 19                   | 115          |
| 2            | 500                 | 10       | 17               | 14           | 18                   | 100          |
| 2            | 2500                | 06       | 09               | 07           | 12                   | 58           |
| 3            | 100                 | 19       | 22               | 17           | 23                   | 108          |
| 3            | 500                 | 16       | 20               | 16           | 21                   | 108          |
| 3            | 2500                | 12       | 19               | 13           | 18                   | 95           |
| 4            | 100                 | 15       | 17               | 15           | 18                   | 110          |
| 4            | 500                 | 10       | 17               | 11           | 17                   | 95           |
| 4            | 2500                | 08       | 10               | 08           | 13                   | 80           |
| 5            | 100                 | 17       | 22               | 15           | 24                   | 110          |
| 5            | 500                 | 13       | 20               | 13           | 20                   | 91           |
| 5            | 2500                | 12       | 12               | 12           | 19                   | 90           |
| 6            | 100                 | 17       | 20               | 16           | 24                   | 95           |
| 6            | 500                 | 15       | 19               | 15           | 23                   | 61           |
| 6            | 2500                | 13       | 19               | 13           | 23                   | 59           |
| 7            | 100                 | 10       | 15               | 10           | 14                   | 30           |
| 7            | 500                 | 06       | 11               | 03           | 11                   | 11           |
| 7            | 2500                | 03       | 10               | 03           | 11                   | 2            |
| 8            | 100                 | 08       | 13               | 06           | 13                   | 65           |
| 8            | 500                 | 06       | 12               | 06           | 12                   | 45           |
| 8            | 2500                | 03       | 10               | 02           | 07                   | 12           |
| 9            | 100                 | 07       | 18               | 06           | 13                   | 48           |
| 9            | 500                 | 05       | 13               | 04           | 12                   | 25           |
| 9            | 2500                | 05       | 12               | 04           | 12                   | 12           |
| 10           | 100                 | 17       | 22               | 18           | 24                   | 98           |
| 10           | 500                 | 16       | 20               | 16           | 19                   | 80           |
| 10           | 2500                | 13       | 28               | 11           | 13                   | 80           |
| 11           | 100                 | 17       | 22               | 19           | 23                   | 100          |
| 11           | 500                 | 15       | 20               | 17           | 29                   | 85           |
| 11           | 2500                | 12       | 18               | 11           | 13                   | 80           |
| 12           | 100                 | 11       | 16               | 06           | 18                   | 80           |
| 12           | 500                 | 06       | 14               | 04           | 14                   | 31           |
| 12           | 2500                | 02       | 06               | 03           | 06                   | 6            |
| 13           | 100                 | 04       | 11               | 18           | 24                   | 35           |
| 13           | 500                 | 03       | 07               | 09           | 14                   | 28           |
| 13           | 2500                | 03       | 07               | 06           | 13                   | 15           |

## EXAMPLE 21

A high sensitivity silver halide emulsion containing 1.8 mole % of AgI and 98.2 mole % of AgBr was divided into several portions. To these portions were added respectively the compounds reported in Table 4. The resulting emulsion samples were then spread on a polyester support previously thinly coated with gelatin containing iron powder. Samples of the resulting films were developed in Ferrania R-14 developer (Example 19) for 3' at 20°C. The capacity of the compounds to inhibit spot formation was evaluated by counting the number of the spots per unit area in several areas of each sample. Results are reported in Table No. 4.

TABLE 4

| Compound No. | $\mu\text{M/M AgX}$ | Number of Spots | Solvent Used                    |
|--------------|---------------------|-----------------|---------------------------------|
| test         | —                   | 90              |                                 |
| 14           | 500                 | 15              | $\text{H}_2\text{O}$            |
| 15           | do.                 | 16              | $\text{H}_2\text{O}$            |
| 16           | do.                 | 10              | $\text{H}_2\text{O}$            |
| 17           | do.                 | 18              | $\text{C}_2\text{H}_5\text{OH}$ |
| 1            | do.                 | 9               | $\text{H}_2\text{O}$            |
| 2            | do.                 | 22              | DMF                             |
| 3            | do.                 | 6               | $\text{H}_2\text{O}$            |
| 4            | do.                 | 15              | DMF                             |
| 5            | do.                 | 12              | $\text{H}_2\text{O}$            |
| 6            | do.                 | 11              | DMF                             |
| 7            | do.                 | 0               | $\text{C}_2\text{H}_5\text{OH}$ |
| 8            | do.                 | 0               | $\text{C}_2\text{H}_5\text{OH}$ |
| 9            | do.                 | 0               | DMF                             |
| 10           | do.                 | 12              | $\text{C}_2\text{H}_5\text{OH}$ |
| 11           | do.                 | 16              | $\text{C}_2\text{H}_5\text{OH}$ |
| 12           | do.                 | 14              | $\text{C}_2\text{H}_5\text{OH}$ |
| 13           | do.                 | 0               | $\text{C}_2\text{H}_5\text{OH}$ |

What we claim is:

1. A silver halide photographic emulsion containing a fog inhibiting amount of an azodicarbonamidine salt.

2. The emulsion of claim 1 wherein said azodicarbonamidine salt is characterized by the formula

wherein  $\text{R}_1$ ,  $\text{R}_2$ ,  $\text{R}_3$  and  $\text{R}_4$  independently are hydrogen, alkyl or aryl, and  $\text{X}$  represents an equivalent of anion.

3. The emulsion of claim 2 wherein the anion of said azodicarbonamidine salt is chloride, nitrate, sulfate or picrate.

4. The emulsion according to claim 1 wherein said azodicarbonamidine salt is contained therewithin in a concentration of from about 0.1 to about 2.5 millimoles per gram atom of silver.

5. The silver halide photographic emulsion according to claim 1 wherein said azodicarbonamidine salt is a salt of  $\text{N},\text{N}'$ -dimethyl-azodicarbonamidine.

6. The photographic emulsion according to claim 5 wherein said azodicarbonamidine salt is the nitrate or picrate salt.

7. A photographic element which includes a silver halide emulsion layer, said emulsion layer containing a

fog inhibiting amount of an azodicarbonamide salt, or said emulsion layer having an adjacent layer containing a fog inhibiting amount of an azodicarbonamide salt.

8. The photographic element of claim 7 wherein said azodicarbonamide salts is incorporated in said emul-

sion layer.

9. The photographic element according to claim 7 wherein said azodicarbonamide salt is in a layer adjacent said silver halide emulsion layer.

5

\* \* \* \* \*

10

15

20

25

30

35

40

45

50

55

60

65